

May 21, 1940.

G. S. FULCHER

2,201,723

CAST REFRACTORY BLOCK AND METHOD OF PRODUCING THE SAME

Filed Sept. 28, 1937



Fig. 6.



Inventor  
GORDON S. FULCHER

May 21, 1940  
Densley, Cole & Garner  
Attorneys

## UNITED STATES PATENT OFFICE

2,201,723

CAST REFRACTORY BLOCK AND METHOD  
OF PRODUCING THE SAMEGordon S. Fulcher, Louisville, Ky., assignor to  
Corhart Refractories Company, Louisville, Ky.

Application September 28, 1937, Serial No. 166,155

4 Claims. (Cl. 49—79)

One of the serious problems attending the casting of refractory materials from the melts thereof is the formation of pipes in the casting during the cooling of the material from its casting temperature (approximately 1800° C.) to its setting temperature. This pipe tends to form at the top of the cast block where the font was located in the casting, destroying the smooth finish of the casting at that point and creating a cavity which may form the center of attack if molten glass enters it. The present invention has for its object to convert the space formed by the contraction from a pipe such as has hitherto been formed, into a cavity entirely enclosed within the surface of the block, and this I accomplish by turning the block around a horizontal axis during the period of its setting. My invention, therefore, consists of such process as well as the product resulting therefrom.

Referring to the accompanying drawing in which corresponding parts are designated by corresponding marks of reference,

Figure 1 represents in section a mold by which my invention may be carried out.

Figure 2 shows such a mold after it has been filled with the molten material and closed.

Figures 3 and 4 represent the mold in a rocking frame constructed in accordance with this invention.

Figure 5 is a diagrammatic view of the rocking frame shown in Figures 3 and 4 with means for rocking the same.

Figure 6 is a diagrammatic section through a block embodying my invention and having two enclosed cavities.

The mold 11 of a well known construction is enclosed in a metal flask 12, the mold having a top plate 13 with a font 14 thereon. After the mold is filled with the molten material the top plate 13 and the font 14 are removed and replaced by a refractory slab 15, and a cover 16 is clamped thereon with a layer of insulation 16a interposed between them.

The flask is now clamped in a rocking frame consisting of two wheels 17, each having a framework 18 built within its periphery and provided with screws 19 to clamp the opposite ends of the flask, which during the time it is being fixed in position may rest on a stand 20.

Upon removing the stand from beneath the flask the wheels may be rolled along a suitable track. As a convenient device for this purpose the wheels may run on an inclined track 21 being pulled up the track by ropes 22 and a windlass 23, and after being pulled up for half a turn the wheels may be released to roll back to the lower position. Obviously, other means may be resorted to for rocking or rotating the casting on a horizontal axis. The motion around this axis may be and preferably is slow (say, one complete

cycle in ten minutes) to permit the molten material to be spread over all sides of the mold by the movement of the box and to solidify thereon and without washing the solidified material out of place. Under such treatment the molten material will solidify in layers on all six sides of the flask (including what was the top thereof), thus locating the cavity, which is necessarily formed by the contraction of the molten material, more or less in the center of the casting.

For certain purposes it is desirable that the central section of the casting be solid. I can accomplish this, according to this invention, by rocking the horizontal axis of the block during solidification through an angle of 45° to one side 15 to a 45° angle on the other once every five or ten minutes during cooling. In this operation the central section, which is filled with the liquid at all times, will become practically solid. In Figure 6 the dotted lines indicate the thickness of the wall at successive stages of cooling. It is believed that for certain purposes the location of the cavities in the ends of the block is preferable to any other situation.

Instead of rocking the block back and forth 25 during all or a substantial part of the time it is solidifying, it may be simply turned on a horizontal axis after the casting and permitted to stay stationary in this turned position with one end higher than the other during the solidification, whereby the cavity resulting from the contraction of the material will be found in the upper end.

Having thus described my invention, what I claim is:

1. The hereinbefore described method of casting and solidifying a refractory block from molten material which comprises pouring the molten material into a mold having the intended shape and size of the cast article and thereafter 40 during solidification, turning the casting and mold around a horizontal axis.

2. The hereinbefore described method of casting and solidifying a refractory block from molten material which comprises pouring the 45 molten material into a mold having the intended shape and size of the cast article and thereafter during its solidification slowly rocking the casting and mold around a horizontal axis.

3. A cast block of refractory material, having 50 the cavities resulting from the contraction of such material during cooling located at opposite ends of the block.

4. A cast block of refractory material, and having the cavity resulting from the contraction of 60 such material during solidification substantially symmetrical in respect to an axis of the block which was horizontal during the casting and entirely enclosed.

GORDON S. FULCHER. 60